

Patented June 14, 1927.

1,632,419

# UNITED STATES PATENT OFFICE.

TUDOR REES SIMPSON, OF JOHANNESBURG, TRANSVAAL, SOUTH AFRICA, ASSIGNOR  
TO MINERALS SEPARATION NORTH AMERICAN CORPORATION, OF NEW YORK, N. Y.,  
A CORPORATION.

## CONCENTRATION OF METALLIFEROUS ORES.

No Drawing. Application filed May 27, 1926, Serial No. 112,129, and in the Union of South Africa June 9, 1925.

This invention comprises improvements in or relating to the concentration of metalliferous ores.

According to the present invention a process of froth-flotation concentration is characterized by effecting flotation of an aqueous pulp of ore containing metalliferous matter and gangue in the presence of a protective organic colloid (for example starch, glue, 10 gelatine or the like) the amount of which is sufficient to inhibit flotation of gangue constituents of the ore but insufficient to inhibit flotation of desired metalliferous constituents of the ore.

15 The present invention relates to the separation of the metalliferous constituents of ores from gangue minerals of such a nature as to tend to float in substantial quantities under the usual conditions of flotation and 20 which are therefore particularly difficult to eliminate from concentrates containing the metalliferous constituents during the operation of flotation processes. The insoluble silicate gangues known as talcose gangues 25 constitute one type of such gangue minerals. Useful application of the invention has been found in the flotation concentration of values from norite rock. It has also been found to be highly effective in the flotation of gold 30 ores of the type which is generally known as "talcose".

The invention has been found to be specially beneficial in the treatment of ores such as those of the Lydenburg district, which 35 carry sulphide minerals and platinum. The colloid may be added during the grinding of the ore, during the primary flotation of the ore, or during the retreatment of the products of the primary concentration.

40 As herein illustrated the invention comprises the addition of organic protective colloids (for example starch, glue, gelatine or the like) to an aqueous pulp of ore containing an organic sulphhydric compound such 45 as an alkaline xanthate so that it is present during the flotation with the colloid. In this way marked improvement in separation of values from gangue may be secured in some cases.

50 The colloid in liquid form may be added before or during the agitation operation. Its effect is apparently more or less to retard the flotation of all the constituents of the ore.

It must therefore be added in a regulated amount, as otherwise not only the undesired, 55 but also the desired, constituents may be rendered unfloatable.

The amount of the colloid employed may be determined experimentally, as is usual with the reagents employed in the froth-flotation process, and a simple preliminary test will suffice to indicate the proper amount to be used with any particular ore.

55 The following is one example illustrative of the method of carrying the invention into effect:—

The ore was a norite sulphide ore from the Lydenburg district of the Union of South Africa. It assayed 0.21% of nickel, 0.11% of copper and 2.1 dwts. per ton of 70 platinum group metals. The ore was first crushed so that 95% passed through a screen of 60 meshes per lineal inch and was made into an aqueous pulp having a ratio of water to solids lying between 4:1 and 5:1. A preliminary concentration was effected by submitting the pulp to flotation in a sub-aeration machine with the addition of 0.5 lb. of cresol per ton of ore and 0.2 lb. of sodium xanthate per ton of ore. The concentrate 75 amounting to about one-fifth of the crude ore contained a considerable amount of readily floatable gangue material; it was diluted with water to form a pulp having a water-to-solid ratio of 10:1 and a starch solution 80 was added at the rate of 0.25 lb. of starch per ton of the original crude ore. Flotation was then effected in a sub-aeration machine without the addition of any other reagent. In the result a concentrate was obtained 85 which assayed 73.7 dwts. of platinum metals per ton and contained 7.68% of nickel and 3.75% of copper. The recovery of platinum was 89% and the tailings contained only traces of nickel and copper. The amount of the final concentrate was about 2.1% of the original ore. The gangue in this example 90 was talcose.

I claim:

1. The process of concentrating a material carrying floatable mineral and gangue which consists in agitating a pulp of the suitably ground material with a mineral-frothing agent in the presence of an organic sulphhydric compound and an organic protective colloid substance adapted to selec- 100  
105

tively inhibit the flotation of a large proportion of normally floatable gangue material, and separating a froth carrying a large proportion of a mineral present.

6. 2. The process of concentrating a material carrying floatable mineral and gangue which consists in agitating a pulp of the suitably ground material with a mineral-frothing agent in the presence of a xanthate and an 10 organic protective colloid substance adapted to selectively inhibit the flotation of a large proportion of normally floatable gangue material, and separating a froth carrying a large proportion of a mineral present.

15. 3. The process of concentrating a material carrying floatable mineral and gangue which consists in agitating a pulp of the suitably ground material with a mineral-frothing agent in the presence of an organic sulph- 20 hydric compound and starch in such proportion as selectively inhibits the flotation of a large proportion of normally floatable gangue material, and separating a froth carrying a large proportion of a mineral present.

25. 4. The process of concentrating a material carrying floatable mineral and gangue which consists in agitating a pulp of the suitably ground material with a mineral-frothing 30 agent in the presence of a xanthate and starch in such proportion as selectively inhibits the flotation of a large proportion of normally floatable gangue material, and separating a froth carrying a large proportion 35 of a mineral present.

40. 5. The process of concentrating a material carrying floatable mineral and gangue which consists in agitating a pulp of the suitably ground material with a soluble mineral-frothing agent in the presence of a xanthate and with starch in such proportion as selectively inhibits the flotation of a large proportion of normally floatable gangue material, and separating a froth carrying a large 45 proportion of a mineral.

50. 6. The process of obtaining a relatively rich concentrate from a mineral-containing material carrying a substantial amount of normally floatable insoluble silicate gangue which consists in agitating a pulp of the suitably ground material with an organic sulphhydric compound and an organic protective colloid substance so as to yield a froth concentrate relatively rich in a mineral 55 of the material and relatively free from said silicate, and separating the froth concentrate.

60. 7. The process of obtaining a relatively rich concentrate from a mineral-containing material carrying a substantial amount of normally floatable insoluble silicate gangue which consists in agitating a pulp of the suitably ground material with a xanthate and an organic protective colloid substance 65 so as to yield a froth concentrate relatively

rich in a mineral of the material and relatively free from said silicate, and separating the froth concentrate.

8. The process of concentrating ores carrying a substantial amount of normally floatable insoluble silicate gangue which consists in agitating a pulp of the ore with a mineral-frothing agent so as to yield a mineral-bearing froth carrying a relatively large proportion of a mineral of the ore accompanied by a large proportion of said silicate, separating the froth, agitating a pulp of the froth concentrate with a xanthate and an organic protective colloid substance so as to yield a froth concentrate relatively 80 rich in said mineral and relatively free from said silicate, and separating the froth concentrate.

9. The process of obtaining a relatively rich concentrate from a mineral-containing 85 material carrying a substantial amount of normally floatable insoluble silicate gangue which consists in agitating a pulp of the suitably ground material with a xanthate and with a small proportion of starch so as to yield a froth concentrate relatively rich in a mineral of the ore and relatively free from said silicate, and separating the froth concentrate.

10. The process of concentrating ores carrying a substantial amount of normally floatable insoluble silicate gangue which consists in agitating a pulp of the ore with a mineral-frothing agent and with an organic sulphhydric compound so as to yield a mineral-bearing froth carrying a relatively large proportion of a mineral of the ore accompanied by a large proportion of said silicate, separating the froth, agitating a pulp of the froth concentrate with the further addition 105 of starch so as to yield a froth concentrate relatively rich in said mineral and relatively free from said silicate, and separating the froth concentrate.

11. The process of concentrating ores carrying a substantial amount of normally floatable insoluble silicate gangue which consists in agitating a pulp of the ore with a mineral-frothing agent and with a xanthate so as to yield a mineral-bearing froth carrying a relatively large proportion of a mineral of the ore accompanied by a large proportion of said silicate, separating the froth, agitating a pulp of the froth concentrate with the further addition of starch so as to 115 yield a froth concentrate relatively rich in said mineral and relatively free from said silicate, and separating the froth concentrate.

12. The process of concentrating a material carrying a floatable mineral and normally floatable talcose gangue which consists in agitating a pulp of the suitably ground material in the presence of a mineral-frothing agent and a xanthate and starch so as 120

to yield a mineral-bearing froth relatively poor in the talcose gangue, and separating the froth.

13. The process of concentrating an ore carrying floatable mineral and normally floatable talcose gangue which consists in agitating a pulp of the suitably ground ore in the presence of a mineral-frothing agent and a xanthate so as to yield a mineral-bearing froth carrying a large proportion of a mineral accompanied by a large proportion

of said talcose gangue, separating the froth concentrate, agitating the froth concentrate with the further addition of starch so as to yield a mineral-bearing froth relatively rich in said mineral and relatively poor in said talcose gangue, and separating the froth.

In testimony whereof he has signed his name to this specification at Johannesburg, Transvaal Province of the Union of South Africa, this 23rd day of April, 1926.

TUDOR REES SIMPSON.